

Oct. 19, 1943.

R. G. WALTENBERG

2,332,416

BIMETAL

Filed Nov. 4, 1940



INVENTOR

Romaine G. Waltenberg

BY

Lucie, Don, Marjorie and Edmunds

ATTORNEYS

## UNITED STATES PATENT OFFICE

2,332,416

## BIMETAL

Romaine G. Waltenberg, Roselle, N. J., assignor  
to The H. A. Wilson Company, Newark, N. J.,  
a corporation of New Jersey

Application November 4, 1940, Serial No. 364,124

2 Claims. (Cl. 297—15)

This invention is concerned with thermally-responsive bimetals employed for determination or control of temperature or temperature change in heating devices and the like. The invention provides improved steel bimetals of high corrosion resistance and great sensitivity so that they are capable of deflecting markedly and exerting great force per unit of weight with small temperature change.

Thermally-responsive bimetals, hereinafter referred to simply as "bimetals," comprise two or more metal members (sometimes called "components" or "sides") having different rates of expansion under the influence of heat and joined together in a unitary structure that changes shape as it is heated or cooled. Thus, the bimetal may comprise two steel strips of different composition and expansibilities bonded together side by side. When the bimetal is heated, its two sides expand unequally so that it bends in an arc.

Bimetals frequently are exposed to severe oxidizing conditions (for example, when immersed in water) and in such cases their life is short unless they offer high resistance to corrosion. Heretofore customary bimetals in which both high-expanding and low-expanding sides are steels are capable of withstanding relatively high temperature without acquiring permanent set, but heretofore such bimetals have not afforded both high corrosion resistance and high sensitivity—at least to an adequate extent. In order to obtain high corrosion resistance in steel bimetals, it has been necessary to sacrifice sensitivity and, conversely, steel bimetals of high sensitivity have been relatively susceptible to corrosion.

Failure of bimetals through corrosion may come about because the individual sides have insufficient resistance to the oxidizing influences to which they are exposed or because of galvanic action between the sides, especially at the bond between them. Thus, metals which are resistant to corrosion if taken by themselves may fail to resist corrosion if taken together in the bimetal.

As a result of my investigations, I have developed a steel bimetal having both great sensitivity and high corrosion resistance and which can be employed under conditions that are too severe for heretofore customary bimetals. The components of the bimetal of my invention individually have high resistance to corrosion and are compatible with each other so that the effect of galvanic action is minimized and the bond between components is corrosion-resistant. Moreover, the rates of the expansion of the compo-

nents with temperature are so different that the bimetal is very sensitive, deflecting markedly with small changes in temperature and exerting great force per unit of weight. Both components of the bimetal of my invention are nickel steels, the low-expanding component being of the "Invar" type, i. e., a steel in which the sum of nickel and cobalt contents is very high and the high-expanding side being an austenitic steel containing substantially less nickel than the low-expanding side but with appreciable proportions of chromium and molybdenum. Thus, the low-expanding side may be a steel with a nickel content ranging from about 30% to about 38% and a cobalt content ranging from about 2% to about 10%, the combined nickel and cobalt content being of the order of 40%. The high-expanding side may be a steel containing chromium in proportions ranging from 7-12% plus sufficient nickel to render the steel austenitic (say 17-20%) and a substantial proportion of molybdenum (say of the order of 3%).

The bond between the components of my bimetal may be and preferably is autogenous, i. e., the two components are fastened together directly without an intermediate layer. The bond may be formed in accordance with heretofore customary practice, for example, by welding together billets of the respective components disposed side by side and rolling out the resulting laminated mass to the desired thickness. Such a bond is strong and lasting, if, as in the case of my bimetal, the sides themselves and the bond are proof against oxidizing influences.

"Invar" type steels are well-known and, as indicated above, are characterized by a low rate of expansion with temperature. Invar type steels, considered generally, may have a combined nickel and cobalt content (if cobalt is present) ranging from 30-55%. The cobalt content of the Invar type steel component of the bimetal of my invention should lie in the range of about 2% to about 10% and the nickel content preferably should lie in the range of 30% to 38%. The combined nickel and cobalt content of the low-expanding component should be well within the general Invar range of 30-55% and for best results should lie in the range of 36-42%. The low-expanding component may and, in fact, should contain a substantial proportion of chromium, say 5% to 8%. The balance of metal in the low-expanding component is essentially iron, i. e., elemental iron with small proportions of usual commercial ingredients, such as carbon, phosphorus, sulfur, silicon and manganese. It is, of

course, desirable to keep these ingredients at a minimum and in particular the manganese content should not be permitted to exceed 1% and preferably should be below  $\frac{1}{2}$ %.

The high-expanding side of my bimetal is an austenitic steel as distinguished from a steel of the Invar type, that is to say the alloy ingredients employed in the high-expanding side, such as nickel and chromium, are not present in proportion greatly exceeding that required for preserving austenitic structure at room temperature and, of course, at the temperature of service. Both chromium and nickel tend to preserve austenitic structure. A straight nickel steel is austenitic in character with a nickel content of about 25%. The nickel content may be reduced substantially and still preserve austenitic structure of the steel if chromium is present. Thus, such steel containing 3% chromium is austenitic if it also contains 21-22% nickel. If the chromium content is raised to 9%, the nickel content may be reduced to about 18%. Consequently, a high-expanding component of the bimetal of my invention which contains 7-12% chromium (the preferred proportion) requires nickel in proportion ranging from about 17% to about 20%. The high-expanding component, however, must also contain substantial proportions of molybdenum (say 2% to 4%). The balance of the metal present in the low-expanding side is essentially iron and should be relatively free of ingredients such as carbon, phosphorus and silicon. However, manganese may be present in proportions of the order of 1%, although such a high manganese content is not essential.

The preferred range of ingredients in both the low-expanding side and the high-expanding side of the bimetal of my invention is indicated on the following table:

Table I

| Ingredients | Low-expanding component     | High-expanding component |
|-------------|-----------------------------|--------------------------|
| Ni.         | Per cent by weight<br>20-38 | 17-20                    |
| Cr.         | 6-8                         | 7-12                     |
| Mn.         | Less than 1                 | 1 or less                |
| Co.         | 2-10                        | 2-4                      |
| Mo.         |                             |                          |
| NI+CO.      | 36-42                       |                          |

A specific example of a bimetal of my invention possessing both great sensitivity and long life, due to high corrosion resistance of the components both individually and collectively, is as follows:

Table II

| Ingredients | Low-expanding component                | High-expanding component |
|-------------|----------------------------------------|--------------------------|
| Ni.         | Per cent by weight<br>31 $\frac{1}{2}$ | 17 $\frac{1}{2}$         |
| Cr.         | 6                                      | 9 $\frac{1}{2}$          |
| Mn.         | 1 $\frac{1}{2}$                        | 1                        |
| Co.         | 8                                      |                          |
| Mo.         |                                        |                          |
| NI+CO.      | 39 $\frac{1}{2}$                       | 3                        |

The properties of the bimetal of Table II (which is characteristic of all the bimetals of my invention) may best be described with reference to the accompanying drawing in which sensitivity is shown by two graphs. Thus, curve A is a

plot of deflection in inches against temperature in degrees Fahrenheit of a bimetal strip of the analysis given in Table II. The strip was .050 inch thick by .25 inch wide by 3.16 inches long and prior to test had been heat-treated for one hour at 650° C. Curve B on the graph illustrates flexibility of this bimetal strip.

The flexibility (F) of a bimetal, as defined by the American Society for Testing Materials, is the change in curvature per unit temperature per unit thickness. It is customary to consider flexibility in the terms of a constant K which depends upon the differences in thermal expansion, in ratio of elastic moduli and in thickness of the components (sides) of the bimetal, the relationship between F and K and other factors being expressed by the equation:

$$F = 2K = \frac{\left(\frac{1}{R_2} - \frac{1}{R_1}\right)t}{T_2 - T_1}$$

It will be seen that flexibility or K is a measure of the sensitivity of a bimetal to temperature change at a given temperature level. The values for the K of the bimetal of the Table II at different temperatures are plotted on the graph as curve B. Referring to this curve, it will be observed that the maximum flexibility of the bimetal occurs for a temperature range up to about 300° F. and the bimetal is particularly sensitive up to this temperature. At temperatures higher than 300° F., the flexibility decreases.

As indicated above, curve A on the graph shows the deflection of the bimetal at various temperatures. It will be observed that deflection increases rapidly and more or less constantly to a temperature of about 450° F.-500° F. At higher temperatures deflection increases at a substantially lower rate, so from the standpoint of deflection, the preferred operating range of the bimetal is below about 500° F.

To summarize, the temperature range of useful deflection of the bimetal of Table II is from about -50° C. to about +500° F. The temperature range of maximum sensitivity of the bimetal, as indicated by curve B, is from +50° F. to about +300° F. The K value of the bimetal over the temperature range of maximum sensitivity is about .0000053. The bimetal has an electrical resistivity at 70° F. of about 400 ohms per sq. mil.-ft., and its modulus of elasticity in pounds per square inch is about 25,000,000.

The bimetal of Table II (like the others of this invention) is strongly resistant to corrosion and need not be protected with a coating or plating even when in use under severe oxidizing conditions. Its temperature deflection rate is substantially greater than that of bronze-steel bimetals now in use and exerts substantially greater force per unit of weight for changes in temperature.

The bimetal has a long life and does not fail by splitting, which occurs in other bimetals in which galvanic action with or without oxidizing influence brings about failure of the bond between the components.

I claim:

1. A steel bimetal adapted to change shape as its temperature is changed and comprising two steel components of different expansibilities welded directly together, the individual components and the bond between them being strongly resistant to corrosion by galvanic action between the components, the low-expanding component and the high-expanding component being respec-

tively of the Invar and the austenitic types and having the following analyses:

| Low-expanding component |                    | High-expanding component |                    |
|-------------------------|--------------------|--------------------------|--------------------|
| Ingredients             | Per cent by weight | Ingredients              | Per cent by weight |
| Co.....                 | 2-10               | Mo.....                  | 2-4                |
| Co and Ni.....          | 30-55              | Cr.....                  | 7-12               |
| Cr.....                 | (1)                | Ni.....                  | 17-20              |
| Fe.....                 | (2)                | Fe.....                  | (a)                |

<sup>1</sup> Effective proportions up to 8 per cent.

<sup>2</sup> Balance.

2. A steel bimetal adapted to change shape as its temperature is changed and comprising two steel components of different expansibilities welded directly together, the individual compo-

nents and the bond between them being strongly resistant to corrosion by galvanic action between the components, the low-expanding component and the high-expanding component being respectively of the Invar and the austenitic type and having the following analyses:

| Low-expanding component |                    | High-expanding component |                    |
|-------------------------|--------------------|--------------------------|--------------------|
| Ingredients             | Per cent by weight | Ingredients              | Per cent by weight |
| Co.....                 | 2-10               | Mo.....                  | 2-4                |
| Co and Ni.....          | 36-42              | Cr.....                  | 7-12               |
| Cr.....                 | 5-8                | Ni.....                  | 17-20              |
| Fe.....                 | Balance            | Fe.....                  | Balance            |

ROMAINE G. WALTENBERG.